

E. N. MORRILL.

METHOD OF AND APPARATUS FOR SMELTING TIN,  
APPLICATION FILED NOV. 27, 1917.

1,271,200.

Patented July 2, 1918.

2 SHEETS—SHEET 1.



E. N. MORRILL.

METHOD OF AND APPARATUS FOR SMELTING TIN.  
APPLICATION FILED NOV. 27, 1917.

1,271,200.

Patented July 2, 1918.

2 SHEETS—SHEET 2.



Inventor  
Edmund N. Morris.  
By his Attorneys  
Newell & Neal.

# UNITED STATES PATENT OFFICE.

EDMUND N. MORRILL, OF WARREN, NEW HAMPSHIRE, ASSIGNOR TO ANDES EXPLORATION & SMELTING CORPORATION, A CORPORATION OF DELAWARE.

## METHOD OF AND APPARATUS FOR SMELTING TIN.

1,271,200.

Specification of Letters Patent. Patented July 2, 1918.

Application filed November 27, 1917. Serial No. 202,176.

To all whom it may concern:

Be it known that I, EDMUND N. MORRILL, a citizen of the United States, residing at Warren, Grafton county, New Hampshire, have invented certain new and useful Improvements in Methods of and Apparatus for Smelting Tin, of which the following is a clear, full, and exact description.

This invention relates to a process and apparatus for smelting tin ore electrically and the apparatus comprises an electric incandescent furnace of special construction and although designed more particularly for the carrying out of the present process, yet its advantageous features may well be employed for other purposes.

In the smelting of tin ore, it is desirable to prevent as far as possible, the vaporization of the reduced tin and, therefore, one of the objects of this invention is to smelt the ore under a pressure and at a temperature which will minimize said vaporization. Of course a very slight vaporization of tin will take place from the molten tin metal but no great vaporization will take place unless the tin reaches its boiling point, approximately 1600° C. In the working of the present process, I prefer to employ a molten slag bath as the resistant between two separated electrodes in contact therewith to furnish the heat within the furnace necessary for smelting, for the reason that by proper adjustment of the distance between said electrodes and of the voltage of the electric current, the temperature of the molten material in the furnace may be very carefully regulated so as not to exceed 1600° C.

The crucible within the furnace is preferably kept closed against the admission of air and the pressure within said crucible may be controlled by choking the discharge of gases through the exit flue. The examination of the gases passing out of the exit flue will be one way of determining, by the absence or presence of the well recognized whitish smoke, whether the temperature in the furnace is excessive.

In carrying out the present process, I also prefer to employ a comparatively large current at low pressure. For example, the amperage may run from 1,000 to 2,200 amperes and the pressure of the current is preferably from 20 to 110 volts. The depth of the slag bath and distance between the electrodes in contact therewith are suitably adjusted, so

far as possible, to maintain the voltage and amperage between these figures. The temperature of the molten material within the furnace is, as before stated, slightly below the boiling point of tin and approximately 60 1500° C and in order to maintain this temperature uniform, so far as possible, under conditions of tapping out slag and molten tin and introducing fresh charges, the pressure of the electric current must be capable 65 of gradual adjustment through a wide range, and this may be accomplished through any suitable system of voltage regulation.

A further object of the present invention is to provide an electric furnace which will 70 not leak tin and with crucible walls of such refractory material as will not disintegrate under the destructive and decomposing tendencies of the molten slag and metal. As is well known, tin, lead and analogous metals 75 are extremely penetrating when in a molten condition and it is a common experience with tin furnaces heretofore employed, that after being in use for some time, the walls become soaked with tin, and furthermore, 80 considerable tin has been lost by its penetrating through the walls and base of the furnace into the earth. To overcome this defect of prior furnaces, the present furnace is built and supported upon a solid block or 85 base of concrete with raised border walls which is practically impervious to the tin and serves as a collecting basin therefor.

Further objects and advantages of the present process and apparatus will become 90 apparent in the following specification which describes a suitable and preferred embodiment of the invention and the novel features thereof will be pointed out in the appending claims.

Referring to the drawings:

Figure 1 is a vertical section through the furnace along line 1—1 of Fig. 2.

Fig. 2 is another vertical section through the furnace along line 2—2 of Fig. 1; the 100 sections shown in Figs. 1 and 2 being at right angles to one another.

Fig. 3 is a detail section through the crucible showing a typical condition of the material therein at separate levels.

Referring more particularly to the drawings, 1 indicates the foundation and supporting base of the furnace which is made of a solid block of concrete, slightly sunk 105 into the earth as shown and with raised 110

- border walls 3. Upon the base 1 the outer walls 4 of the furnace are built up from suitable fire brick. Within the walls 4 is inclosed the crucible 5, made of magnesite brick forming a lining therefor and topped overhead with a suitable arch, which may be of fire brick. The sides of the arches are supported by beams of railroad iron 7, and I beams of railroad iron 8 are embedded in the concrete base 1, of the furnace extending fore and aft therethrough, as shown so as to be tied to similar I beams 9, running over the top of the furnace. The I beams are connected at their ends as shown in Fig. 10 by tie rods 10, having turn buckles 11 therein for taking up any looseness thereof as it occurs in the expansion and contraction of the walls of the furnace. The furnace is also suitably tied together transversely by transverse rods 12, embedded in the top and bottom of the furnace respectively, and with their protruding ends passing through vertical I beams 14, as shown in Fig. 1.
- 15 25 An eductor or flue for exhaust gases is shown at 15, communicating with the top of the crucible and passing outwardly through the furnace to the stack 16. A choke damper 17 is mounted in the eductor flue so as to choke the discharge of the exhaust gases therethrough and to thereby maintain the required pressure within the crucible. A plurality of feed holes 18, preferably four in number, are provided through 30 the arch of the crucible and top of the furnace, by which fresh charges of ore and material may be introduced into the crucible and it is understood that normally, during the running of the furnace, the feed 35 holes are closed by plug covers 19.
- 30 45 The upper electrode 20 of the furnace, preferably a carbon stick, is shown as entering centrally through the top of the crucible and with its lower end dipping slightly into the molten slag, the level of which is indicated at 21. The floor of the crucible 5, is stepped down to a central gutter 22, and at the bottom of the gutter 22, is exposed the lower electrode 23. The lower electrode is 50 also preferably of carbon and is carried upon the end of a suitable conducting element 24, embedded in the fire brick at the base of the furnace extending outwardly thereof for connection to an offset conductor 25. It will be noted by reference to Fig. 2 that said conductor 25 is offset upwardly within the walls of the furnace and is extended to the exterior of said wall by arm 26, at a point above the level 27<sup>a</sup> of the 55 molten metal within the crucible. The purpose of this is to prevent the leakage of molten metal outwardly of said furnace through the packed joint between said conductor and the walls of the furnace.
- 60 65 The conducting arm 26 for the lower electrode is

60 65 electrode is suitably connected to a current carrying cable 27<sup>a</sup>. The upper electrode 20 is adjustably supported within a water jacketed clamp 28 hung from chains 29, said chains and clamp serving as the electrical conductor for the upper electrode. The chains may be raised or lowered from an upper support (not shown) to dip the electrode 20 more or less into the bath of slag 21, and likewise the clamp 28 may be loosened by bolts 29 for extending the carbon stick 20 therethrough as the same is consumed. 30, 31 indicate the water circulation pipes for the water jacket of said clamp 28. A typical condition of the materials within the crucible is illustrated more clearly in Fig. 3, wherein the level of the molten metal which gravitates to the bottom of the crucible is shown at 27 and the level of molten slag above the metal is shown at 21. 70 Above the molten slag are separate heaps of a freshly introduced charge 18<sup>a</sup> and 18<sup>b</sup>, said charges being introduced through the feed holes 18. It is to be understood that when first introduced, the charge even though containing some materials which might be heavier than the molten slag, nevertheless, since these are thoroughly mixed with lighter elements, the charge as a whole or at least a substantial part of it 80 will normally float on top of the slag bath until smelted down. Immediately, however, the heat of the slag bath starts the chemical reactions which take place between the several elements of the charge for reducing the metal of the ore. In other words, the metal of the ore is gradually fluxed and melted out of the charge and gravitates through the slag bath to the level of the molten metal at the bottom of the crucible. 85

90 95 The magnesite walls of the crucible are backed on all four sides with water cooling bosh plates 39, which extend vertically above and below the molten material within said crucible. The water circulating pipes 100 for said bosh plates are shown at 40. The purpose of said water cooled bosh plates, of course, is to prevent the disintegration of the crucible walls due to the intense heat of the molten metals to which it is subjected. The 105 purpose of water jacketing the clamp 28 is to prevent the undesirable heating both of itself and of the electrode 20. 110

115 120 On a level with the bottom of the crucible gutter is a tap hole 30 for the molten metal, which opens into what is known as a "cinder monkey" 31, shown as comprising a wrought iron member with flaring mouth 32, and water jacketed walls 33. Pipes 34<sup>a</sup>, 35<sup>a</sup> are the water circulation pipes for the water 125 jacket 33 of said cinder monkey. A similar tap hole 34, is provided slightly above the floor of the crucible as shown in Fig. 1, for tapping out slag and a similar cinder monkey 35 is also provided for the slag tap 130

hole and is likewise water jacketed at 36, and provided with water circulating pipes 37, 38.

The furnace is operated and the present process is preferably carried out as follows: Starting with the furnace cold, a small quantity of coke is introduced in the bottom of the crucible around the lower electrode and the upper electrode is lowered to come 10 in contact with said coke, so as to give a closed circuit for the electrical current through the coke to the lower electrode. The current is then sent through the electrodes at a pressure of about 30 volts, the 15 amperage at this time being rather high on account of the low resistance furnished by the coke. As the coke begins to glow red hot, easily fusible slag is introduced to furnish a slag bath within the crucible. The 20 slag as it melts is slowly increased in depth by the introduction of new charges, and the upper electrode is gradually pulled away from the lower electrode until the resistance is increased sufficiently to cut down the am- 25 perage to about 1500 amperes. The molten bath of slag thus formed is preferably heated to a temperature of about 1500° C., whereupon it is ready for the introduction of the ore to be smelted. The charge is then 30 fed in small quantities through one or more of the feed holes described, the quantity of each charge thus introduced being smaller than the volume of molten material already in the furnace so as not to perceptibly cool 35 down said molten material. The charge of ore and reducing materials is made up in approximately the following proportions:

|                                                 |                   |
|-------------------------------------------------|-------------------|
| 60% concentrated tin<br>(SnO <sub>2</sub> ) ore | 1000 pounds       |
| Slag                                            | 100 pounds        |
| Lime (CaO)                                      | 35 to 50 pounds   |
| Silica (SiO <sub>2</sub> )                      | 50 to 70 pounds   |
| Coal                                            | 125 to 150 pounds |

45 Each charge upon coming in contact with the molten slag is heated sufficiently to bring about the chemical reactions necessary for reducing the tin ore, and the molten tin gradually sinks to the bottom of the crucible 50 around the lower electrode. The lighter slag and other impurities rises and forms a bath above the molten metal.

During the working of the process, the voltage is regulated to maintain the required 55 current for generating the necessary heat within the furnace and is preferably maintained around 50 volts. Sometimes, however, it may be necessary to quickly raise the voltage as high as 110 or lower it to 20, 60 in order to take care of special conditions. The molten metal is tapped off at frequent intervals through the lower tap hole and cinder monkey 30, 31, and the slag is also tapped off at suitable intervals through the 65 upper tap hole 34 and 35. The upper car-

bon electrode 20, is adjusted up or down when required to keep its lower end just dipping within the slag bath and to maintain the proper resistance between the electrodes, as is required for a current of about 70 1500 amperes under a pressure of about 50 volts. During the running of the furnace a slight pressure is maintained within the same by choking the discharge of exhaust gases through the eductor 15, so that a 75 temperature of 1500° C. within the furnace will quickly reduce the ore, without causing any appreciable vaporization of the molten metal.

It is to be understood, of course, that both 80 the process heretofore particularly described and also the apparatus as shown and described may be varied as to exact proportions or details of construction without departing from the spirit and scope of the in- 85 vention as claimed.

What I claim as new is:—

1. The process of smelting tin ore in an electric incandescent furnace, which consists in forming a molten slag bath in said furnace by its resistance to an electric current 90 passing therethrough, introducing at intervals into said bath, a charge of tin ore, slag and reducing materials, each freshly introduced charge being smaller in quantity than 95 the volume of said molten material already in said furnace, and maintaining the temperature of said bath approximately uniform and slightly below the boiling point 100 of tin.

2. The process of smelting tin ore in an electric incandescent furnace, which consists in forming a molten slag bath in a furnace closed to the atmosphere by its resistance to an electric current passing therethrough, introducing at intervals into said bath, a charge of tin ore, slag and reducing materials, each freshly introduced charge being smaller in quantity than 105 the volume of said molten material already in said furnace, and maintaining the temperature of said bath approximately uniform and slightly below 110 the boiling point of tin.

3. The process of smelting tin ore in an electric incandescent furnace, which consists in forming a molten slag bath in said furnace by its resistance to an electric current 115 passing therethrough, introducing at intervals into said bath, a charge of tin ore, slag and reducing materials, each freshly introduced charge being smaller in quantity than 120 the volume of said molten material already in said furnace, and maintaining the temperature of said bath approximately uniform and slightly below the boiling point 125 of tin and choking the discharge of gases from said furnace to retard the vaporization of said tin.

4. The process of smelting tin ore in an electric incandescent furnace, which consists 130

- in forming a molten slag bath in said furnace by its resistance to an electric current passing therethrough, introducing at intervals into said bath, a charge of tin ore, slag and reducing materials in approximate proportion of 60% concentrated tin ore—1000 lbs., slag—100 lbs., lime CaO—35 to 50 lbs., silica  $SiO_2$ —50 to 70 lbs., coal—125 to 150 lbs., each freshly introduced charge being smaller in quantity than the volume of said molten material already in said furnace, and maintaining the temperature of said bath approximately uniform and slightly below the boiling point of tin.
- 15 5. The process of smelting tin ore in an electric incandescent furnace, which consists in forming a molten slag bath in said furnace by its resistance to an electric current passing therethrough, introducing at intervals into said bath, a charge of tin ore, slag and reducing materials, each freshly introduced charge being smaller in quantity than the molten metal material already in said furnace, and maintaining the temperature of said bath approximately uniform and slightly below the boiling point of tin by a current varying from 1500 to 2200 amperes and under pressures of from 35 to 60 volts.
- 20 6. The process of smelting tin ore in an electric incandescent furnace, which consists in forming a molten slag bath in said furnace by its resistance to an electric current passing therethrough between separated electrodes in contact with said bath, introducing at intervals into said bath, a charge of ore, slag and reducing materials, each freshly introduced charge being smaller in quantity than the material already in said furnace, maintaining the temperature of said bath approximately uniform and slightly below the boiling point of tin and tapping off said slag and said reduced metal at intervals but never in greater quantity than that which will keep the electrodes dipping 25 in said bath.
- 30 7. An electric incandescent furnace comprising a crucible lined with magnesite brick, said lining being surrounded by a backing of fire-brick and the whole sup-

ported upon a solid base of concrete having 50 a raised border wall to prevent leakage of molten material from said furnace into the earth, the hearth of said crucible being surrounded by water-cooled plates located between said magnesite lining and fire-brick 55 backing.

8. An electric incandescent furnace comprising a crucible lined with magnesite brick, said lining being surrounded by a backing of fire-brick and the whole supported upon a solid base of concrete having 60 a raised border wall to prevent leakage of molten material from said furnace into the earth, the hearth of said crucible being surrounded by water-cooled plates located adjacent 65 said magnesite lining, tap holes for said slag and for said molten metal at different levels, each of said tap holes having outwardly flaring mouths and being surrounded with a water jacket.

70 9. An electric incandescent furnace closed on all sides, comprising a crucible for containing molten material and lined with refractory material and having supporting walls, an upper electrode projecting through 75 the top of said furnace and a lower electrode at the bottom of said crucible, said lower electrode entering the side wall of said furnace at a point above the level of molten material within said crucible and being offset 80 downwardly within said side wall to project into the crucible at the bottom thereof.

10. An electric incandescent furnace, comprising a crucible for containing molten material and having upper and lower electrodes, the lower electrode being exposed through the bottom of said crucible for electrical contact with said molten material and being offset laterally and upwardly within 90 the wall of said crucible so as to extend outwardly through the said wall thereof at a point above the level of the molten material in said crucible.

Signed at New York, N. Y., this 15th day 95 of November, 1917.

EDMUND N. MORRILL.